



US005985060A

# United States Patent [19]

Cabrera et al.

[11] Patent Number: **5,985,060**[45] Date of Patent: **Nov. 16, 1999**[54] **GAS GENERANT COMPOSITIONS  
CONTAINING GUANIDINES**[75] Inventors: **Raul Cabrera**, Tampa; **Cezary Grzelczyk**, Lakeland, both of Fla.[73] Assignee: **Breed Automotive Technology, Inc.**, Lakeland, Fla.[21] Appl. No.: **09/122,545**[22] Filed: **Jul. 25, 1998**[51] Int. Cl.<sup>6</sup> ..... **C06B 31/12; C06B 29/22**[52] U.S. Cl. ..... **149/62; 149/76**

[58] Field of Search ..... 149/62, 76

[56] **References Cited**

## U.S. PATENT DOCUMENTS

|           |         |               |          |
|-----------|---------|---------------|----------|
| 3,031,347 | 4/1962  | Philipson     | .        |
| 3,929,530 | 12/1975 | Niles         | 149/84   |
| 3,939,018 | 2/1976  | Sayles        | 149/19.1 |
| 4,971,640 | 11/1990 | Chi           | 149/19.9 |
| 5,035,757 | 7/1991  | Poole         | 149/46   |
| 5,467,715 | 11/1995 | Taylor et al. | 102/289  |
| 5,500,059 | 3/1996  | Lund et al.   | 149/19.1 |

|           |        |                 |         |
|-----------|--------|-----------------|---------|
| 5,529,647 | 6/1996 | Taylor et al.   | 149/2   |
| 5,531,941 | 7/1996 | Poole           | 264/3.4 |
| 5,739,460 | 4/1998 | Knowlton et al. | 102/324 |

## OTHER PUBLICATIONS

Ebling et al., "Development of gas generators for fire extinguishing", Propellants, Explosives, Pyrotechnics (Jul. 1997) vol. 22 (3), p. 170-175.

Primary Examiner—Charles T. Jordan

Assistant Examiner—Aileen J. Baker

Attorney, Agent, or Firm—L. R. Drayer; D. O. Nickey

[57] **ABSTRACT**

The present invention relates to improved non-azide gas generators and methods for their manufacture for use in an automobile gas bag system. This discovery overcomes the problems of moisture and thermal cycling in a non-azide gas generant pellet through the use of at least two fuels selected from guanidine nitrate, nitroguanidine, triaminoguanidine nitrate, diaminoguanidine nitrate and monoguanidine nitrate and an oxidizer system comprising mixtures of strontium nitrate, sodium nitrate and ammonium perchlorate.

**10 Claims, 2 Drawing Sheets**







FIG-2A



FIG-2B



FIG-3

## GAS GENERANT COMPOSITIONS CONTAINING GUANIDINES

The present invention relates to non-azide gas generants containing guanidines that are useful for inflating an airbag in a vehicle occupant protection system.

### BACKGROUND OF THE INVENTION

Automobile airbag systems have been developed to protect vehicle occupants in the event of a crash by rapidly inflating a cushion or bag between a vehicle occupant and the interior of the vehicle. The inflated airbag absorbs the vehicle occupant's energy to provide a gradual, controlled deceleration and provides a cushion to distribute body loads and keep the occupant from impacting the hard surfaces of the vehicle interior.

The use of such protective gas-inflated airbags to cushion vehicle occupants in crash situations is now widely known and well documented. The requirements of a gas generant used in an automobile airbag inflator are very demanding. The gas generant must have a burning rate such that the airbag is inflated rapidly (within approximately 30-100 milliseconds) and the burning rate must not vary over long term storage (aging and/or thermal cycling) or as a result of shock and vibration encountered during the life of the vehicle. The burning rate must also be relatively insensitive to changes in humidity and temperature. When pressed into pellets, wafers, cylinders, discs or whatever shape, the hardness and mechanical strength of the gas generant bodies must be adequate to withstand the conditions to which they will be exposed without any fragmentation or change of exposed surface area. Excessive breakage of the generant bodies will lead to system failure where, for example, an undesirable high pressure condition will be created within the inflator, possibly resulting in catastrophic rupture of the inflator housing.

The gas generant must efficiently produce a relatively cool, non-toxic, non-corrosive gas which is easily filtered to remove solid and liquid combustion by-products. This filtering is needed to preclude damage to the inflatable airbag or injury to the occupant of the automobile. These requirements limit the applicability of many otherwise suitable chemical compositions, shapes and configurations from being used in automotive airbag inflators. Gas generants can also be used for fire extinguishing. Recently, a number of companies have begun using the gases produced by solid energetic or pyrotechnique materials for fire extinguishing.

An important parameter relating to gas generants is physical stability of the gas generant pellet. As mentioned above, physical forces, such as vibration, can abrade or crack the gas generant pellets. This damage is unacceptable as the surface area is increased and thus the ballistics (rate of combustion) are altered. Ballistics can also be altered through the absorption of water and thermal cycling. It is known that most non-azide based gas generants, especially 5-aminotetrazole, are hygroscopic and soften upon heating. These changes cause the gas generant pellet to degrade or crumble. This change in surface area can result in catastrophic failure of the inflator housing due to excessive pressure build up in the housing at the time of ignition.

A source of water for degradation of a generant pellet is the gas generant itself. Many non-azide gas generants are prepared by an aqueous mixing process. Water is used to mix the non-azide fuel, oxidizer, and other components of the gas generant composition. The majority of the water is removed during a drying step, however, at least 1% by weight and

sometimes as high as 5% by weight water still remains in the generant composition. This drying step is expensive and dangerous. Any method that would allow the gas generant to be prepared without the use of water would be readily accepted by the industry.

In its broadest aspect, the present invention overcomes the previously described problems through the use of guanidines as the fuel and an oxidizer system comprising strontium nitrate and ammonium perchlorate. In addition, the invention, as it relates to the inflator housing, comprises the use of a metal ribbon with a plurality of apertures and a segment of expanded metal that is rolled into a coil and used as a filter to trap combustion products. The following discussion of the background art will assist the artisan in understanding the advancements that the present invention brings to the industry.

### BACKGROUND ART

U.S. Pat. No. 5,035,757 to Poole teaches gas generant compositions devoid of azides which yields solid combustion products which are easily filtered. This patent provides a good discussion of formulating non-azide based gas generants. This patent also teaches that alkaline earth and cerium nitrate oxidizers are hygroscopic and are difficult to use effectively.

U.S. Pat. No. 5,500,059 to Lund et al. teaches a gas generant composition comprising an oxidizer and anhydrous 5-aminotetrazole as the fuel. This patent points out that 5-aminotetrazole (5-AT) is generally in the monohydrate form and that gas generating compositions based upon hydrated tetrazoles have unacceptably low burning rates. Specifically, this patent teaches a method for the production of gas generant pellets comprising the steps of: a) preparing a water slurry of an oxidizer and hydrated 5-aminotetrazole; b) drying the slurred material to a constant weight; c) pressing said material into pellets in hydrated form; and d) drying said pellets such that the gas generating material is in anhydrous or substantially anhydrous form. This patent teaches that if the material is pressed into pellets while in the anhydrous form, the pellets are observed to powder and crumble, particularly when exposed to a humid environment. This reference goes on to state that after the final drying step, it is desirable to protect the pellets from exposure to moisture. It is further suggested that the pellets be placed within a sealed container, or coated with a water impermeable material.

U.S. Pat. No. 5,467,715 to Taylor et al. relates to a gas generant composition that contains, as a fuel, a mixture of triazoles or tetrazoles with a minor portion of a water soluble fuel and an oxidizer component wherein 20 weight % of the oxidizer component is a transition metal oxide.

U.S. Pat. No. 5,529,647 to Taylor et al. teaches a gas generant for airbags which comprises between 2 and 45 weight % of a tetrazole or triazole compound; from 50-75 weight % of an oxidizer such as ammonium nitrate, ammonium perchlorate, transition metal oxides and mixtures thereof; from 0.5 to about 30 weight % of alumina fibers; and between about 1 and 10 weight % of a binder such as molybdenum disulfide, graphite, nitrocellulose, calcium stearate and mixtures thereof.

U.S. Pat. No. 5,531,941 to Poole teaches an azide-free gas generant composition that comprises a mixture of triaminoguanidine nitrate (TAGN) as the fuel and phase stabilized ammonium nitrate (PSAN) as the oxidizer. Poole teaches that one of the major problems with the use of ammonium nitrate (AN) is that it undergoes several crystalline phase

changes. One of these phase changes occurs at approximately 32° C. and is accompanied by a large change in crystal volume. If a gas generant containing a significant amount of AN is thermally cycled above and below the phase transition temperature, the AN crystals expand and contract resulting in crumbling and cracking of the gas generant pellet. Poole points out that this is totally unacceptable in a gas generant because the burning characteristics would be altered such that the inflator would not operate properly or might even blow up because of the excess pressure generated.

U.S. Pat. No. 3,031,347 to Philipson teaches to solid propellant materials useful in rocket or jet propulsion motors. The slow burning propellant composition of Philipson uses an oxidizer selected from ammonium perchlorate, ammonium nitrate and mixtures thereof at concentrations of from 45 to 72 weight %. The Philipson composition also uses 5–22 weight % of an oxygen rich additive selected from the group consisting of guanidine nitrate, nitroguanidine, cellulose nitrate and mixtures thereof; and 23–36 weight % of a polymerized resin fuel. This reference fails to make any suggestion that an automobile airbag gas generant can be prepared from a mixture of at least two fuels selected from guanidine nitrate (GN), nitroguanidine (NG), triaminoguanidine nitrate (TGN), diaminoguanidine nitrate (DGN) and monoguanidine nitrate (MGN); an oxidizer system which is a mixture of alkali metal nitrates, alkaline earth metal nitrates and ammonium perchlorate; and a catalyst selected from copper chromite, iron oxide and mixtures thereof.

U.S. Pat. No. 3,929,530 to Niles teaches a pyrotechnic composition for colored smoke production and for the distribution of pesticides, fumigants, herbicides and the like. The pyrotechnic disseminating composition taught in this reference employs an amino-substituted thiourea compound as a fuel; inorganic oxidizers such as alkali metal and ammonium chlorates and perchlorates; combustion catalysts such as chromates, copper salts, metal chromites, ferric oxide and the like; and a compound to be disseminated such as smoke producing organic dyes, tear gas, herbicides, pesticides, psychotomimetic incapacitating agents and the like. While the use of tear gas and herbicides is contraindicated in gas generants for vehicle airbags, the use of fuels such as those suggested (i.e., amino-substituted thioureas) would also not be acceptable as high levels of sulfur containing combustion by-products, such as  $H_2S$  and  $H_2SO_4$ , would be harmful to the vehicle occupants. As such, this patent fails to suggest or disclose the gas generant of the present invention.

U.S. Pat. No. 3,939,018 to Sayles teaches the use of tris(difluoroamino)-methoxyethyl ammonium perchlorate as a substitute for the conventional burning rate catalysts such as ferric oxide, copper chromite and a variety of other ferrocene compounds. The teachings of this patent will not be useful in an automobile gas generant as the presence of fluorine would present a health concern for vehicle occupants.

In a publication by Ebeling et al. entitled, "Development of gas generators for fire extinguishing", *Propellants, Explosives, Pyrotechnics*, (July, 1997) Vol. 22(3), p. 170–175, the authors evaluate the idea of using gases or aerosols produced by solid energetic or pyrotechnique materials for fire extinguishing. The authors considered the class of nitrogen rich, low carbon content compounds, such as NG, TGN and 5-amino-1H-tetrazole. This publication does not suggest that NG be combined with GN, TGN, DGN and/or MGN, ammonium perchlorate and copper chromite to produce a gas generant which has excellent

thermal stability, good gas production properties and produces a low level of toxic gases upon combustion.

#### SUMMARY OF THE INVENTION

In accordance with one aspect of the present invention the gas generant composition comprises: (a) a fuel component which is used at a level between about 45 and about 70 weight %, which comprises a mixture of at least two fuels selected from the group consisting of guanidine nitrate (GN), nitroguanidine (NG), triaminoguanidine nitrate (TGN), diaminoguanidine nitrate (DGN) and monoguanidine nitrate (MGN); and (b) an oxidizer component which is used at a level of between about 25 and about 50 weight %, which comprises a mixture of the alkali metal nitrates, alkaline earth metal nitrates, and ammonium perchlorate.

The catalyst may preferably be selected from copper chromite, iron oxide, and mixtures thereof and may comprise from 0.1 to 1.0 weight % of the composition.

In a preferred embodiment, the fuel component comprises a mixture of NG and GN; the oxidizer component comprises a mixture of strontium nitrate (SN), ammonium perchlorate (AP) and sodium nitrate (NaN); and the catalyst is copper chromite (CuCr).

In a yet more preferred embodiment, the gas generant composition comprises 10–20 weight % NG, 35–50 weight % GN, 5–15 weight % strontium nitrate (SN), 15–25 weight % ammonium perchlorate (AP), 5–25 weight % sodium nitrate (NaN) and 0.1–0.3 weight % copper chromite. In a still more preferred embodiment, the composition comprises 14–17 weight % of NG, 40–43 weight % of GN, 7–10 weight % SN, 21–24 weight % AP, 10–13 weight % NaN and about 0.2–0.3 weight % copper chromite (CuCr).

Further important aspects of the inventive gas generant include: the quantity of harmful gases that are generated upon combustion is below specified limits; a high gas output (at least 700 mols/kg of generant); low toxicity of basic materials and reaction products; sufficient chemical and thermal stability; low sensitivity to friction and impact; low cost of production; availability of basic materials; processing on a large scale is possible; and potential for recycling.

One aspect of the invention relates to a method of producing the gas generant composition without the use of water. In general, the process comprises the dry blending of all the components and then pelletizing. For example, in a dry blender, i.e., a tubular mixer, the fuels and the oxidizers such as AP, NaN and SN, are mixed together until a homogeneous blend is achieved. This dry blend then has added to it the CuCr. The product is then pelletized using conventional equipment and techniques to produce pellets of from 5–500 mgs. It is preferred that the fuels, oxidizers and catalyst be substantially anhydrous.

The gas generants of the invention, while primarily directed to use in vehicle occupant restraint systems, can also be applied to fire extinguishing systems. Further, the generants of the invention are particularly useful in the all-chemical-generated gas system. The generants are also very useful in hybrid systems which feature a gas generant unit in combination with a stored gas unit.

#### BRIEF DESCRIPTION OF THE DRAWINGS

The features of the invention which are believed to be novel are set forth with particularity in the appended claims. The present invention, both as to its structure and manner of operation, may best be understood by referring to the

following detailed description, taken in accordance with the accompanying drawings in which:

FIG. 1 is an exploded view of an inflator used in the tests described herein and employing the inventive filter system;

FIG. 2A is a top plan view of one embodiment of the metallic ribbon used to prepare the filter coil according to the invention;

FIG. 2B is a top plan view of a second embodiment of the metallic ribbon; and

FIG. 3 is a side view in cross section of the inflator taken along line 3—3 of FIG. 1.

#### BRIEF DETAILED DESCRIPTION OF THE INVENTION

The gas generant formulations used in this invention are formulated from the guanidine family of fuels such as guanidine nitrate (GN), triaminoguanidine nitrate (TAGN) and the like. The fuel component will typically comprise between about 45 and about 70 weight %, more preferably between 50 and 60 weight %, of the gas generant composition, while the oxidizer system will typically comprise between about 35 and about 50 weight %, more preferably between 40 and 50 weight %, of the gas generant composition. Processing aids, such as silicon dioxide, may also be used in formulating the gas generant pellets. Those skilled in the art understand that depending upon the particular oxidizers and fuels utilized, certain processing aids have beneficial properties over others.

The fuel useful in the gas generant of the present invention is a mixture of at least two guanidine fuels selected from guanidine nitrate (GN), nitroguanidine (NG), triaminoguanidine nitrate (TAGN), diaminoguanidine nitrate (DAGN) and monoguanidine nitrate (MGN). Guanidine or iminourea ( $\text{CH}_5\text{N}_3$ ) has the structural formula:



Guanidine is soluble in water and alcohol, volatile and strongly alkaline. It forms many salts, e.g., nitrate and the like. Nitroguanidine is a white crystalline powder which is usually manufactured from calcium carbide via calcium cyanamide, dicyandiamide and guanidine nitrate which is converted to nitroguanidine by action of concentrated sulfuric acid. Nitroguanidine has the structural formula:



Oxidizers useful in the gas generant compositions include ammonium perchlorate and the alkali metal and alkaline earth metal nitrates such as strontium nitrate and sodium nitrate. The preferred oxidizer system is a mixture of strontium nitrate, sodium nitrate and ammonium perchlorate. Ammonium perchlorate is important to the gas generant of the invention due to its gaseous decomposition and lack of particulate production. The potential problem of HCl generation may be overcome through the use of copper chromite and/or iron oxide as a catalyst and/or the sodium from the sodium nitrate. One aspect of the invention is the discovery that AP, which is a component that the industry has a propensity to avoid due to HCl generation, is useful in the

inventive gas generants. As set forth in the Examples, the gas generants of the invention produce barely detectable levels of chloride containing gases.

The ratio of oxidizer to fuel in the inventive gas generant is adjusted such that the amount of oxygen allowed in the equilibrium exhaust gases is from zero to 2 or 3% by volume, and more preferably from zero to 2.0% by volume.

The gas generant composition may optionally contain up to about 1.0 weight %, typically between about 0.1 and about 0.3 weight %, of iron oxide, copper chromite or mixtures thereof as catalysts. Copper chromite (CuCr) has known properties as a catalyst. It is a mixed oxide of copper and chromium obtained by igniting copper ammonium chromate under controlled conditions. Barium is frequently added to prevent poisoning of the catalyst, however, the CuCr used in the present invention is preferably free of barium. Copper chromite is principally used for the reduction of carboxyl groups (e.g., ketones to alcohols, and esters to alcohols). The preferred level of copper chromite in the inventive composition is about 0.25 weight %. The iron oxide ( $\text{Fe}_2\text{O}_3$ ) useful in the inventive compositions may be obtained by all the usual methods. The particle size of the iron oxide and CuCr may vary from about 1 to 10 microns.

The invention will now be described in greater detail by way of specific examples.

Referring to FIG. 1, there is represented in exploded view, an inflator 10 employed in testing several of the gas generant compositions disclosed herein. A first housing member 12 and a second housing member 22 are attached to one another through "friction or inertia welding". The inflator 10 also comprises an inventive strip filter 14, an enhancer tube 16, a squib with enhancer cup 18 and a room temperature vulcanizing rubber seal 20. A bed of gas generant pellets 30 is disposed between the strip filter 14 and the enhancer tube 16. Metal foil, not shown, lines the annular surface of the first housing 12 covering gas exit portals 34 in the first housing.

With reference to FIGS. 2A and 2B, there is represented two (2) embodiments of the inventive filter strip 14. Both embodiments of the filter strip contain at least three (3) segments wherein the first segment 28 (a.k.a. the inside portion) has two (2) rows of apertures therethrough positioned along each edge of the ribbon, an expanded metal segment 29 and second segment 15 wherein at least one row of apertures are present. FIG. 2A is an embodiment wherein the second segment 15 has two (2) rows of a plurality of apertures 26 therethrough with diameter of about 2.0 mm. FIG. 2B represents a second embodiment where the second segment 15 has a single row of apertures 26 therethrough with a diameter of about 4 mm. The placement of the apertures is important for complete combustion of the generant. The first segment, which is adjacent the generant bed, requires apertures along each edges, while the second or final segment must have the aperture in the center of the ribbon. The size and number of the apertures can be varied to control the desired combustion level (i.e., rate of pressure generation). In use, the filter strip is coiled or rolled into a tubular configuration which is placed inside the inflator 10.

The inventors have discovered that a metallic filter strip or ribbon with a combination of segments with holes and a segment of expanded metal can economically produce a filter that effectively cools the gas and removes particulates and slag generated when the gas generant is burned. The metal from which the filter strip 14 is produced can be any metal with a melting point high enough to survive the combustion of the gas generant. The thickness of the strip

can range from about 0.25 mm to 1.27 mm with about 0.51 mm to 0.76 mm being more preferred, about 0.63 mm being the most preferred.

The length and height of the strip can vary widely depending upon the size and configuration of the inflator housing into which it is placed. Dependent on the size of the housing, the filter strip is designed such that first segment 28 will complete the first turn during the formation of the coil and the expanded metal segment 29 will complete at least two turns of the coil. Preferably, the expanded metal segment 29 will complete at least three turns. The second segment 15 is of such length that it will completely circumferentially cover the outside of the coil.

Another important aspect of the filter strip is that apertures 24 in the first segment 28 are not aligned with, and do not overlay, the apertures 26 in the second segment 15. In the embodiment set forth in FIG. 2A, the apertures 24 are disposed towards the outside edge of segment 28 while the apertures 26 in the second segment 15 are disposed towards the interior. This aspect is important as it aids in creating a tortuous path for the gases. Further, the use of the expanded metal segment provides a large surface area for the capture of particulates and cooling of the gas and also creates a tortuous path for the gases.

As mentioned previously, the expanded metal segment 29 should be long enough to accomplish at least two (2) turns during the formation of the coil. The diamond shaped openings in the expanded metal segment 29 should have a dimension of about 0.04 to 0.12 mm by 0.32 to 0.8 mm. The expanded metal strip can be made by die cut stamping and the apertures can be drilled or stamped out.

FIG. 3 is a cross section of an inflator housing taken along line 3—3 of FIG. 1 except that the squib with enhancer cup

configurations. As those skilled in the art will appreciate, changing the combustion level and temperature will change the CO and NO<sub>x</sub> content of the combustion gas as well as output. As an example, reduction of the combustion temperature by using a coolant, on the one hand, gives disadvantages relating to CO and NO<sub>x</sub> content as well as output levels. On the other hand, at high output temperature, it leads to potential disadvantages with respect to damage to the airbag. Gas generant development should be understood to be a task of balancing contradicting properties in order to fulfill very special requirements.

In addition, it should be considered that reaction behavior of a gas generant, in areas other than basic chemistry, depends on igniting behavior, combustion surface area and design of the inflator housing which influences pressure build-up. Lastly, the design of the inflator housing can influence the properties of the gas generated through pressure build up as a result of filtering capabilities.

## EXAMPLE I

### Preparation of Gas Generant

A one Kg batch of a gas generant composition was formulated according to Table I below. The compositions were prepared by grinding the individual components (when needed, i.e., NaN) to a particle size of less than 100 microns and then all of the components of the generant were sifted and then blended in a Turbula® mixer (manufactured by W.A.B. of Switzerland). Mixing continued for one (1) hour.

TABLE I

| Sample No. | Values in Weight % |                   |                   |                      |                |                 |      |      |
|------------|--------------------|-------------------|-------------------|----------------------|----------------|-----------------|------|------|
|            | Nitro-guanidine    | Guanidine nitrate | Strontium nitrate | Ammonium perchlorate | Sodium nitrate | Nitro-cellulose | DPA* | CuCr |
| 1          | 15                 | 40                | 10                | 22                   | 11             | 2               | 0.1  | —    |
| 2          | 15                 | 40                | 10                | 22                   | 11             | 2               | —    | —    |
| 3          | 15                 | 42                | 10                | 22                   | 11             | —               | —    | —    |
| 4          | 15                 | 41.5              | 10                | 22                   | 11             | —               | —    | 0.5  |
| 5          | 15.5               | 41.5              | 8.8               | 22.8                 | 11.4           | —               | —    | 0.25 |
| 6          | 13.5               | 44                | 9                 | 22                   | 11             | —               | —    | 0.5  |
| 7          | 15                 | 40                | 10                | 22                   | 11             | 2               | 0.1  | 0.25 |

\*DPA diphenylamine

18 is not shown in cross section. The bed of gas generant 36 is not shown for clarity. The inflator housing 10 comprises a first housing member 12 and a second housing member 22 that, in this representative embodiment, are attached by a spin weld 32. Other forms of attachment such as threaded engagement, laser welds and mechanical fixation, are within the scope of the invention. The filtration strip 14 in coiled configuration, is shown as having five (5) turns in FIG. 1. The apertures 24 through the first segment 28 can be in other arrangements than shown, i.e., in a random pattern, provided the apertures 24 are not directly across from the apertures 26 through the second segment. This is required so that the combustion gas must take a tortuous path through the expanded metal to the apertures 26 and then through the exit portals 34.

One additional aspect of the invention is that through subtle changes in the levels of the various components, the combustion temperature and igniting behavior of the generant can be modified to function in a variety of inflator

The material was then pelletized with a rotary pellet press. 50 The pellets were about 5 mm in diameter, 1.8 mm high, weighed about 55 to 65 mg each and had a density of about 1.6 to 1.7 g/cm<sup>3</sup>.

The formed pellets were then loaded into steel inflators of the type shown in FIG. 1. Either about 19 or 23 gms of the 55 pellets were loaded into each of the steel housings. The 19 gm charge of generant was for a 40 liter airbag while the 23 gm charge was for a 60 liter airbag. The burst foil or tape comprises a thin sheet (about 0.005 mm. thick) of stainless steel with an adhesive on one side. The adhesive side of the 60 burst foil is placed against the inside surface of the inflator housing so as to hermetically seal all of the apertures 34. The apertures 34 are exhaust ports for the gases generated by the generant and were about 2.4 mm in diameter for the 40 liter airbag and about 2.5 mm for the 60 liter airbag. The number of apertures 34 was four. The test inflator housing had a total volume of about 88 cm<sup>3</sup>, while the region of the housing located inwardly of the filter and containing the pellets of

gas generating material had a volume of about 46 cm<sup>3</sup> for the 40 liter airbag and about 46 cm<sup>3</sup> for the 60 liter airbag. The inflator also incorporated about 0.9 g of BKNO<sub>3</sub> (a mixture of boron nitrate and potassium nitrate, conventionally used in the industry), as an enhancer and was associated with the squib with enhancer cup **18**.

## EXAMPLE II

## Testing of the Gas Generant

Two (2) assembled inflators containing 19 gms of the inventive gas generant pellets (Sample No. 5) were evaluated in a (100 cubic foot) test chamber fitted with equipment to record the pressure and time profile of the combustion and to analyze the gases exiting the inflator. The amount of particulate or slag produced by the burning generant was also determined using standardized techniques. The inflators were installed into the test chamber and the gas generant pellets were ignited. The temperature of the inflator at firing was about 23° C.  $\pm$  2° C. at a relative humidity of about 43%. Immediately after firing of the inflator, gas samples were withdrawn from the test chamber for analysis by FTIR (Fourier Transform Infrared Spectroscopy).

Airborne particulate production was measured by filtering post ignition air from the test chamber through a fine filter

and measuring the weight gained by the filter. The average total airborne particulate mass for the two (2) tests was 6.85 mg. The average total particulate concentration for the two (2) tests was 68.5 mg/m<sup>3</sup>.

### Gaseous Reaction Products

The test chamber was attached to a vacuum pump, a bubble flow meter, filters and a FT/IR gas analyzer (spectrophotometer). Gas samples were analyzed using an FTIR spectrometer at zero time (before deployment) and at 1, 5, 10, 15 and 20 minute intervals after ignition or via gas chromatography.

The ammonia, benzene, carbon dioxide, formaldehyde, hydrogen chloride, hydrogen cyanide, methane, sulfur dioxide, carbon monoxide (CO), nitric oxide (NO) and nitrogen dioxide (NO<sub>2</sub>) and water vapor levels of the gases produced in the 100 cubic foot test chamber for the two test samples are set forth in Table II. Samples were transferred directly to the FTIR gas cell from the 100 cubic foot test chamber via six feet of  $\frac{1}{4}$  inch OD fluoropolymer tubing.

TABLE II

| Gaseous Effluent Data  |                  |         |              |                  |                 |                |                   |
|------------------------|------------------|---------|--------------|------------------|-----------------|----------------|-------------------|
|                        | Ammonia          | Benzene | Chloride     | Carbon Dioxide   | Carbon Monoxide | Formaldehyde   | Hydrogen Chloride |
| Analysis Method        | FTIR             | FTIR    | Tube         | FTIR             | FTIR            | FTIR           | FTIR              |
| Detection Limit (ppm)  | 5                | 5       | 0.2          | 50               | 10              | 2              | 2                 |
| Analysis Delay (min)   | 0.2              | 0.2     | 30           | 0.2              | 0.2             | 0.2            | 0.2               |
| Sample No. 5 (Test I)  | 1                | ≤5      | ≤5           | *                | 995             | 142            | <2                |
|                        | 5                | ≤5      | ≤5           | *                | 840             | 117            | <2                |
|                        | 10               | ≤5      | ≤5           | *                | 792             | 109            | <2                |
|                        | 15               | ≤5      | ≤5           | *                | 765             | 106            | <2                |
|                        | 20               | ≤5      | ≤5           | *                | 745             | 103            | <2                |
| TWA                    | ≤5               | ≤5      | ≤5           | **               | 811             | 113            | <2                |
|                        | 20               |         |              |                  |                 |                |                   |
| Sample No. 5 (Test II) | 1                | ≤5      | ≤5           | *                | 805             | 107            | <2                |
|                        | 5                | ≤5      | ≤5           | *                | 863             | 108            | <2                |
|                        | 10               | ≤5      | ≤5           | <0.2             | 796             | 100            | <2                |
|                        | 15               | ≤5      | ≤5           | *                | 765             | 96             | <2                |
|                        | 20               | ≤5      | ≤5           | *                | 754             | 94             | <2                |
| TWA                    | ≤5               | ≤5      | ≤5           | **               | 799             | 101            | <2                |
|                        | 20               |         |              |                  |                 |                |                   |
|                        | Hydrogen cyanide | Methane | Nitric Oxide | Nitrogen dioxide | Phosgene        | Sulfur dioxide | Water Vapor       |
| Analysis Method        | FTIR             | FTIR    | FTIR         | FTIR             | Tube            | FTIR           | FTIR              |
| Detection Limit (ppm)  | 2                | 5       | 2            | 0.5              | 0.02            | 5              | 500               |
| Analysis Delay (min)   | 0.2              | 0.2     | 0.2          | 0.2              | 30              | 0.2            | 0.2               |
| Sample No. 5 (Test I)  | 1                | 12      | 19           | 28               | <0.5            | *              | ≤5                |
|                        | 5                | 10      | 16           | 22               | 1.1             | *              | ≤5                |
|                        | 10               | 9       | 14           | 20               | 1.7             | *              | ≤500              |
|                        | 15               | 8       | 14           | 18               | 2               | *              | ≤500              |
|                        | 20               | 8       | 13           | 17               | 2.4             | *              | ≤500              |
| TWA                    | 9                | 15      | 20           | 1.6              | **              | ≤5             | ≤500              |
|                        | 20               |         |              |                  |                 |                |                   |
| Sample No. 5 (Test II) | 1                | 8       | 14           | 25               | <0.5            | *              | ≤5                |
|                        | 5                | 8       | 14           | 24               | 1.4             | *              | ≤5                |
|                        | 10               | 8       | 12           | 22               | 2               | <0.02          | ≤5                |
|                        | 15               | 8       | 12           | 20               | 2.7             | *              | ≤5                |
|                        | 20               |         |              |                  |                 |                |                   |

TABLE II-continued

| Gaseous Effluent Data |   |    |    |     |    |    |      |  |
|-----------------------|---|----|----|-----|----|----|------|--|
| 20                    | 7 | 12 | 18 | 3.1 | *  | <5 | 2780 |  |
| TWA                   | 8 | 13 | 22 | 2   | ** | <5 | 3068 |  |
| 20                    |   |    |    |     |    |    |      |  |

\* Compound was not analyzed at this time interval

\*\* TWA (total weight average) could not be calculated

+ Gas chromatography tube

The results set forth in Table II demonstrate that the gas generators of the present invention produce an acceptable gas for use in vehicle occupant restraint systems. The gas generators of the present invention produce a reasonably clean combustion gas and the pellets of the generant also resist degradation due to moisture and thermal cycling.

Both firings of the inflator demonstrated acceptable bag inflation, peak bag pressure and sustained bag pressure and thus would be useful in a vehicle airbag occupant safety system.

### EXAMPLE III

#### Thermal Stability

To test the thermal stability of the gas generant according to this invention, 1.0 gm of the Sample No. 5 composition from Table I was placed in a petri-dish and then in an oven at 135° C. for two (2) hours. The sample was removed and allowed to cool at room temperature. Inspection of the pellets revealed that no melting of the gas generant composition had occurred and that the pellets were intact and did not evidence any cracking, crumbling or change in shape.

### EXAMPLE IV

#### Termal Stability

In this experiment, 19 gms of Sample No. 5 was placed in an inflator as set forth in Example II. After assembly of the inflator, the unit was placed in an oven at 107° C. for two (2) hours. The inflator was removed from the oven, allowed to cool to room temperature and then fired. The inflator performed similar to the tests set forth in Example II, thus demonstrating the thermal stability of the compositions according to the invention.

### EXAMPLE V

#### Hot Cold Ignition

In this experiment, the ignition characteristics of the gas generant at 90° C., ambient (about 24° C.) and -40° C. was investigated. 19 gms of the generant Sample No. 5 was loaded into the housings. A total of nine (9) inflators were prepared. Three (3) were placed in an oven at 90° C. for two (2) hours and three (3) were placed in a freezer at -40° C. for two (2) hours. Three inflators remained at room temperature. The inflators were fired at their respective soak temperatures in a 60 liter test chamber fitted to measure combustion gases, pressure and particulates. Plots of pressure versus time were recorded. Table III sets forth the maximum chamber pressure, time to maximum pressure and area under the curve for each test.

TABLE III

| Tank Pressure for Ambient, 90° C. and -40° C. Tests |                     |                           |                                |
|-----------------------------------------------------|---------------------|---------------------------|--------------------------------|
| Test                                                | Max. Pressure (psi) | Time to Max Pressure (ms) | Area under the Curve (PSI *ms) |
| Ambient I                                           | 30.1                | 49.8                      | 4672.7                         |
| Ambient II                                          | 29.7                | 51.6                      | 4615.2                         |
| Ambient III                                         | 29.5                | 50.2                      | 4561.3                         |
| 90° C. I                                            | 33.9                | 40.6                      | 5221.7                         |
| 90° C. II                                           | 32.9                | 42.2                      | 5093.1                         |
| 90° C. III                                          | 32.3                | 42.0                      | 4979.0                         |
| -40° C. I                                           | 26.8                | 57.4                      | 4119.4                         |
| -40° C. II                                          | 26.8                | 58.8                      | 4101.0                         |
| -40° C. III                                         | 26.2                | 54.8                      | 4012.3                         |

The data evidence that the gas generant according to the invention provides satisfactory combustion properties over a wide range of temperatures to properly inflate the airbag.

Total particulate production from each test was also collected. Following venting of the tank to the atmosphere, the interior of the 60 liter test chamber was carefully scrubbed and rinsed with deionized water to measure particulate production. The particulate produced by gas generants comprises a mixture of water soluble and insoluble reaction products. The aqueous mixture of the soluble reaction products and the insoluble dust were analyzed to determine total particulate production. Table IV sets forth the insoluble, soluble and total particulates for each run.

TABLE IV

| Particulate Production |                             |                           |             |
|------------------------|-----------------------------|---------------------------|-------------|
| Test                   | Insoluble Particulates (mg) | Soluble Particulates (mg) | Total (mgs) |
| Ambient I              | 217                         | 760                       | 977         |
| Ambient II             | 128                         | 658                       | 786         |
| Ambient III            | 162                         | 727                       | 889         |
| 90° C. I               | 335                         | 1008                      | 1343        |
| 90° C. II              | 363                         | 1041                      | 1404        |
| 90° C. III             | 180                         | 1036                      | 1216        |
| -40° C. I              | 273                         | 819                       | 1092        |
| -40° C. II             | 319                         | 760                       | 1079        |
| -40° C. III            | 271                         | 777                       | 1048        |

The data evidence that the gas generant composition according to the invention produces a relatively clean gas upon combustion; that is, from a 19 gm charge of generant, less than 1.5 gms of solids exit the inflator.

Toxicity testing was also conducted on the ambient firings of the generant and the results are set forth in Table V.

TABLE V

| Test        | Gas Toxicity Testing - PPM |     |                 |                 |                 |      |                 |                  |                   |
|-------------|----------------------------|-----|-----------------|-----------------|-----------------|------|-----------------|------------------|-------------------|
|             | CO                         | NO  | NO <sub>2</sub> | NH <sub>3</sub> | CO <sub>2</sub> | HCl  | Cl <sub>2</sub> | H <sub>2</sub> S | COCl <sub>2</sub> |
| Ambient I   | 3746                       | 467 | 214             | <5 (2.6%)       | <5              | <0.2 | <0.2            | <0.02            |                   |
| Ambient II  | 3513                       | 320 | 325             | <5 (2.6%)       | <5              | <0.2 | <0.2            | <0.02            |                   |
| Ambient III | 3773                       | 253 | 391             | <5 (2.7%)       | <5              | <0.2 | <0.2            | <0.02            |                   |

( ) = value may be inaccurate, exceeds highest calibration standard.

These data indicate that the generant according to the invention produces a gas that is relatively non-toxic and would therefore be useful in the inflation of air bags and as fire extinguishers.

From these experiments and others that are being conducted at the time of the filing of this application, it is clear that the gas generant according to the invention is useful for inflating airbags and can also be used as fire extinguishers. The generants of the invention are virtually unaffected by temperature extremes and possess excellent ignition and combustion properties. Surprisingly, the use of ammonium perchlorate (AP) does not cause a chlorine problem in the combustion gas. This is quite an unexpected result to those skilled in the art.

#### Industrial Applicability

The automobile industry is in search of gas generants that are free of the problems associated with the use of azide gas generants. The industry is also in need of non-azide based generants that have good, long term stability against moisture degradation and thermal cycling degradation. The gas generant compositions of this invention and the process for their manufacture meet these needs. Further, through the use of a novel combination of materials and a unique process of production, the gas generant of the invention produces a very acceptable gas for the inflation of airbags. Further, the gas generants according to this invention would also find use in fire extinguishing systems using solid energetic materials for producing fire extinguishing gases. Although the present invention has been disclosed in connection with a few preferred embodiments thereof, variations and modifications may be chosen by those skilled in the art without departing from the principles of the invention. All of these variations and modifications are considered to be within the spirit and scope of the present invention as disclosed in the foregoing description and defined by the appended claims.

We claim:

1. A gas generant composition comprising:

- (a) a fuel component which is used at a level between 45 and 70 weight %, which comprises a mixture of at least two fuels selected from the group consisting of guanidine nitrate (GN), nitroguanidine (NG), triaminoguanidine nitrate (TAGN), diaminoguanidine nitrate (DAGN) and monoguanidine nitrate (MGN); and
- (b) an oxidizer component which is used at a level of between 25 and 50 weight %, which comprises a mixture of alkali metal nitrates, alkaline earth metal nitrates, and ammonium perchlorate.

2. The gas generant according to claim 1 wherein said catalyst is selected from copper chromite, iron oxide and mixtures thereof.

3. The gas generant according to claim 1 wherein said catalyst is present at a concentration of 0.1 to 1.0 weight % of the composition.

4. The gas generant according to claim 2 wherein: said fuel component comprises a mixture of NG and GN; said oxidizer component comprises a mixture of strontium nitrate (SN), ammonium perchlorate (AP) and sodium nitrate (NaN); and said catalyst is copper chromite (CuCr).

5. The gas generant according to claim 4 wherein:

- (a) said NG is at a concentration of 10–20 weight % and said GN is at a concentration of 35–50 weight %;
- (b) said SN is at a concentration of 5–15 weight %;
- (b) said AP is at a concentration of 15–25 weight %; and said NaN is at a concentration of 5–25 weight %; and
- (d) said CuCr is at a concentration of 0.2–0.3 weight %.

6. The gas generant according to claim 5 wherein:

- (a) said NG is at a concentration of 14–17 weight %;
- (b) said GN is at a concentration of 40–43 weight %;
- (c) said SN is at a concentration of 7–10 weight %;
- (d) said AP is at a concentration of 21–24 weight %;
- (e) said NaN is at a concentration of 10–13 weight %; and
- (e) said CuCr is at a concentration of 0.2–0.3 weight %.

7. The gas generant composition according to claim 1 wherein said composition is prepared by the steps comprising:

- (i) dry blending said fuel component with said oxidizer component until a homogenous blend is achieved;
- (ii) adding said catalyst to said homogenous blend and blending until a second homogenous blend is achieved; and
- (iii) pelletizing said second homogenous blend to produce pellets of from 5–500 mgs.

8. The gas generant composition according to claim 7 wherein: said fuel component comprises a mixture of NG and GN; said oxidizer component comprises a mixture of strontium nitrate (SN), ammonium perchlorate (AP) and sodium nitrate (NaN); and said catalyst is copper chromite (CuCr).

9. The gas generant composition according to claim 7 wherein said fuel, oxidizer and catalyst are substantially anhydrous.

10. The gas generant composition according to claim 1 which additionally comprises at least one component selected from nitrocellulose and diphenylamine.

\* \* \* \* \*